

Aug. 28, 1928.

1,682,067

L. V. CASTO

MARBLEIZING PROCESS  
PROCESS FOR SIMULATING NATURAL PATTERNS  
Original Filed Jan. 24, 1927



FIG.-1



FIG.-2

*Lloyd V. Casto*  
Inventor

*By Bates, Macklin, Gulick & Tare*

Attorneys

Patented Aug. 28, 1928.

1,682,067

# UNITED STATES PATENT OFFICE.

LLOYD V. CASTO, OF DETROIT, MICHIGAN, ASSIGNOR TO OXFORD VARNISH CORPORATION, OF DETROIT, MICHIGAN, A CORPORATION OF MICHIGAN.

## MARBLEIZING PROCESS.

Application filed January 24, 1927, Serial No. 163,200. Renewed March 16, 1928.

REISSUED

This invention is concerned with processes for refinishing the surfaces of materials in imitation of the natural appearance of other dissimilar materials and has for its general object the provision of a novel process for the reproduction of a marble appearance on the surfaces of materials other than marble.

More specifically my invention has for its object the provision of a process for reproducing in natural colors a marble appearance on surfaces of materials other than marble.

Other objects of my invention will hereinafter be set forth in the following description of a preferred manner of fulfilling the steps of my process. The essential characteristics are summarized in the claims.

In the drawings, in Fig. 1, I show a cross-section of a piece of material, the surface of which has been treated to resemble the surface of a marble slab after the manner of my process; and Fig. 2 is a graphic representation of the application of several coatings of pigments to a surface to impart to the surface a marble appearance.

My invention contemplates the use of the photographic method of obtaining a metallic etching through a carbon resist and thereafter the etched plate or roll, as the case may be, has applied thereto pigments of different colors to simulate the natural colors of a marble surface to be imitated. These colors are successively applied to the etched plate or roll and partake therefrom, the marble pattern in natural contour or outline. This is accomplished by the use of a transfer roll and the transfers applied to the surface being treated in a certain color order whereby the applied coatings when brought into superimposed contrast simulate the natural marble surface.

I first obtain a photographic reproduction of the marble surface on either the usual photographic plate or film and from the plate or film I produce a carbon resist, preferably using a screen and the carbon resist thus obtained, is used in a well known manner to reproduce either a zinc etching or electrotype prepared therefrom and having the characteristics of the well known half-tone plate or a photogravure plate or roll. I prefer to use the latter. If it is desired to use a photogravure plate or roll, one step in the photogravure process is omitted, namely, the making of a positive film or plate from the photographic plate or film. This produces a photo-

gravure roll or plate which is in reality the reverse of the usual photogravure roll or plate. When the plate is thus properly etched, it is then ready for use.

I first treat the surface which is to be 60 marbleized with a ground color A simulating in shade as nearly as possible, the natural shades or tones to be found in the grain or cleavage marks of the natural marble which is to be imitated. I then apply to the photogravure plate or roll a pigment or ink resembling in turn as nearly as possible another color to be found in the original marble slab in the grain or cleavage marks thereof. After using a doctor blade to remove the 70 surplus pigment and thereby leaving pigment deposited only in the etched interstices thereof. I remove the pattern thus outlined by the plate with a transfer roll and apply this pattern designated by the reference character B in the drawings, over the first ground coat previously applied to material to be treated by rolling the transfer roll thereover.

I then apply, after the coating which has 80 been applied in the form of a transfer, has had sufficient time to dry, to the photogravure roll or plate a pigment of still another color resembling in tone the general or dominating color tone of the marble slab to be imitated 85 or reproduced and after using the doctor blade to remove the surplus pigment, I transfer a second pattern in this different color from the plate to the surface being treated, but apply this second pattern designated as 90 C, and which in outline is the same as the first pattern B previously applied, to the surface but out of registration with the contour of the first pattern B. The second application produces an unusual result, in that 95 portions of the ground color and the second color will show through the last applied color at the grain or cleavage veins of the pattern and where the various colors are superimposed there is a variation in tonal effect simulating to a striking degree the varying but natural colors of the original marble slab.

Referring again to Fig. 2 it will be noted that when the two transfers overlay as at D the tone is deepened but this depth of tone 105 will vary in accordance with the variation in the tones of the respective transfers, each of which may vary throughout its surface; and also there will be variations from the initial pigment color of the respective trans- 110

fers for example at E and E' in accordance with the degree of showing of the color of the ground coating A through the transfers. The graphic representation shown in Fig. 2 however, is considerably exaggerated in that only small areas of ground color will be unobscured in the actual reproductions. A protective transparent coating F of varnish or lacquer may be applied to impart to the treated surface the glossy appearance of polished marble.

This process, as will be readily understood, can be used for the application of more than two colors which will show at places on the surface unblended, while at other places where the pattern contours completely superimpose the composite color will vary in tonal depth. This result can be obtained as suggested by either the use of a photogravure half tone or electrotype printing surface derived through the use of the process of producing printing surfaces by photographic methods.

I claim:

25 1. A process for decorating surfaces which includes the use of an etched plate or roll made from a photographic resist, by first treating the surface to be decorated with an underlying or ground coating of pigment, applying the pigment to the etched plate or roll of a color simulating one of the natural grain colors of the marble, transferring the pigment from the plate or roll to the surface to be finished, drying said transferred pattern, applying to the etched plate or roll a second pigment coating and removing said coating therefrom by a resilient roll and thereafter superimposing the transfer pattern over the previously transferred pattern but out of register therewith.

2. A process for simulating marble surfaces on the surfaces of materials other than marble comprising etching a photogravure plate or roll by using a photographic negative plate or film obtained by photographing a marble slab forming a carbon resist from the photographic negative, then using the positive carbon resist thus formed to form a photogravure plate or roll whereby the plate or roll thus formed may be utilized to form pigment transfers of more than one color to be applicable in superposed application relation.

3. A process of reproducing a marble appearance on a hard surface comprising using an etched printing surface prepared from a positive carbon resist of the marble surface to be simulated by applying pigment to the etched surface, removing the pigment from the etched surface by the use of a resilient roll, transferring the reproduced pattern on the resilient roll to the surface to be finished, drying said transferred pattern, applying a different colored pigment to the etched pattern, removing the pigment from the etched

pattern by the use of the resilient roll, and superimposing this pattern of a different colored pigment over the previously transferred pattern whereby marbleizing contrast is effected on the surface to be decorated.

4. A process of reproducing a marble appearance on a hard surface comprising using an etched printing surface prepared from a positive carbon resist of the marble surface to be simulated by applying pigment to the etched surface, removing the pigment from the etched surface by the use of a resilient roll, applying a light shade ground coat to the surface to be finished, transferring the reproduced pattern on the resilient roll to the light shade surface, applying a different colored pigment to the etched pattern, removing the pigment from the etched pattern by the use of the resilient roll, and superimposing this pattern of the different colored pigment over the previously transferred pattern.

5. A process of reproducing a marble appearance on a hard surface comprising using an etched printing surface prepared from a positive carbon resist of the marble to be simulated by using the etched plate or roll thus formed to make pigment transfers of more than one color and separately applying the transfers to the surface to be finished with the transfers of varying colors out of register.

6. A process of reproducing a marble appearance on a hard surface comprising using an etched printing surface prepared from a positive carbon resist of the marble surface to be simulated to make transfers of different colors, applying a light shade ground coat to the surface to be finished, then applying a transfer taken from the etched surface of said plate or roll of a different tone than the ground coat.

7. A process of reproducing a marble appearance on a hard surface comprising using an etched printing surface prepared from a positive carbon resist of the marble surface to be simulated to make pigment transfers of more than one color, coating the surface to be grained with a light ground color, and applying the transfers to the light ground surface with the transfers of varying colors out of register.

8. A process for reproducing a marble appearance on a hard surface comprising using an etched printing surface prepared from a positive carbon resist of the marble surface to be simulated by using the etched plate or roll to make transfers of different colors, applying a ground coat to the surface to be finished, then applying a transfer taken from the etched surface of said plate or roll of a darker tone than the ground coat and then applying a second transfer of a still darker tone.

9. A process of reproducing a marble appearance on a hard surface comprising using

- an etched printing surface prepared from a positive carbon resist of the marble surface to be simulated by using the etched plate or roll thus formed to make pigment transfers of more than one color and applying the transfers to the surface to be finished with the transfers of varying colors out of register, each successive transfer being darker than the previously applied transfer.
10. 10. A process of reproducing a marble appearance on a hard surface comprising using an etched printing surface prepared from a positive carbon resist of the marble surface to be simulated by applying a ground coat to the surface to be finished, then using the etched plate or roll to make transfers of different colors, each successive transfer being made by using a pigment of a darker color than any of the preceding applied pigments.
15. 11. A process for simulating marble surfaces on the surfaces of materials other than marble which includes the steps of producing an etched printing surface by using a photographic negative of the marble surface to form a positive carbon resist and etching a negative printing plate through the positive carbon resist whereby a printing plate or roll is produced which will print in reverse to the usual plate or roll, and whereby the veins or 20 cleavage line formations of the marble surface are indicated by pigment or ink omission during the act of transfer from the printing surface to the surface being finished in simulation of marble.
25. 12. The process of reproducing a marble appearance on a hard surface, comprising using a printing surface derived through the photographic method of printing surface re-
- production which printing surface is negative and used by the application of pigment thereto, then removing the pigment from said printing surface by the use of a resilient roll, transferring the reproduced pattern on the resilient roll to the surface to be finished, applying a different colored pigment to the printing surface, removing the pigment from the printing pattern by the use of a resilient roll, superposing this pattern of a different colored pigment over the previously transferred pattern whereby marbleized contrast is effected on the surface to be decorated.
30. 13. The process of reproducing a marble appearance on a hard surface, comprising using a printing surface derived through the photographic method of reproducing surfaces, the printing surface being negative and used by applying pigments thereto to form pigment transfers of more than one color and separately applying the transfers to the surface to be finished with the transfers of varying colors out of register.
35. 14. A process for simulating marble surfaces on the surfaces of materials other than marble, which includes the step of producing a printing surface derived by the use of the photographic method of printing surface reproduction whereby a negative printing surface is obtained which will print in reverse to the usual plate or roll and thereby define the veins or cleavage lines of the marble surface by pigment or ink omission when said printing surface is used.
- In testimony whereof, I hereunto affix my signature.

LLOYD V. CASTO.